

## UNITED STATES PATENT OFFICE.

SAMUEL E. SHEPPARD AND LEON W. EBERLIN, OF ROCHESTER, NEW YORK, AS-SIGNORS TO EASTMAN KODAK COMPANY, OF ROCHESTER, NEW YORK, A CORPORATION OF NEW YORK.

PROCESS OF REDUCING THE VISCOSITY CHARACTERISTICS OF NITROCELLULOSIC MATERIALS.

No Drawing.

Application filed June 15, 1925. Serial No. 37,405.

To all whom it may concern:

Be it known that we, SAMUEL E. SHEPPARD and LEON W. EBERLIN, a subject of the King of Great Britain and a citizen of the

United States of America, respectively, residing at Rochester, in the county of Monroe and State of New York, have invented certain new and useful Improvements in Processes of Reducing the Viscosity Characteristics of Nitrocellulosic Materials, of which the following is a full, clear, and exact specification.

This invention relates to processes for treating nitrocellulosic materials in such a way as to reduce the viscosity characteristics thereof. One object of the invention is to provide a safe, simple and relatively inexpensive process for treating such materials in order to obtain the desired lower viscosity characteristics. Another object of the invention is to provide a process in which the change in the viscosity characteristics can be effected with sufficient rapidity at room temperature, without the necessity of using heating operations. A further object of the invention is to provide such a process in which the material is readily purified by reason of the practical neutrality of the treating bath. Other objects will hereinafter appear.

In certain industries it is desirable to use solutions of nitrocellulose which have a high concentration of the latter and yet have a low viscosity. It is desirable to provide a safe and relatively inexpensive process for converting the high-viscosity types of nitrocellulose, which are produced in large quantities for many industrial purposes, into nitrocelluloses which have low viscosity characteristics and can, therefore, be made into solutions of the above described type.

We have found that a process having these desirable effects can be carried out by treating nitrocellulosic material with a peroxide solution, preferably one which is substantially neutral. The action proceeds with useful rapidity at room temperature and varies with the concentration of the peroxide, which is usually hydrogen peroxide. The treatment is applicable to nitrocellulose in its various forms and its various associations.

We shall now describe by way of illustration a specific example of our invention, but it will be understood that the latter is not limited to the details, thus given, except as indicated in the appended claims. Nitrocellulosic material, such as pyroxylin waste or photographic film scrap, from which gelatinous material has preferably been removed, or even the original nitrocellulose fibers, are placed, while in comminuted condition in a 3% aqueous solution of hydrogen peroxide of substantial neutrality at room temperature. It is allowed to remain in this bath at room temperature, until the usual tests indicate that the desired lowering of viscosity has taken place. While the time may vary greatly, we have found that a treatment of 24 hours at room temperature, under the above described conditions, produces a very marked reduction in the viscosity characteristics of the nitrocellulose even when the latter is associated with high boiling organic compounds like camphor, butyl alcohol and so forth.

After the action is completed, the bath is drained off from the nitrocellulosic material, and the latter is washed. By reason of the approximate neutrality of the bath, it is very easy to purify the material by washing, there being no large amount of tenaciously held acid or alkali.

Of course, stronger solutions than 3% may be used in order to shorten the time of action. A neutral solution of the ordinary commercial strength and characteristics may be employed. We may even prepare the bath by substantially neutralizing an aqueous solution of sodium peroxide.

Having thus described our invention, what we claim as new and desire to secure by Letters Patent is:

1. The process of treating nitrocellulose which comprises acting thereon with a bath of a peroxide, until its viscosity characteristics are lowered.

2. The process of treating nitrocellulose which comprises acting thereon with a substantially neutral aqueous bath of a peroxide until the viscosity characteristics of the nitrocellulose are reduced.

3. The process of treating nitrocellulose which comprises acting thereon with a sub-

- stantially neutral aqueous solution of hydrogen peroxide, until the viscosity characteristics of the nitrocellulose are reduced.
4. The process of treating nitrocellulose which comprises immersing the same in a substantially neutral aqueous bath of hydrogen peroxide at room temperature until the viscosity characteristics of the nitrocellulose are reduced.
5. The process of treating nitrocellulose which comprises acting thereon with a substantially neutral aqueous bath of hydrogen peroxide, until the viscosity characteristics of the nitrocellulose are lowered, and washing said bath from said material.
6. The process of treating colloidized

nitrocellulose which comprises acting on the same with a bath containing peroxide until the viscosity characteristics of the nitrocellulose are reduced.

7. The process of treating solid colloidized nitrocellulose associated with a high boiling organic compound, which comprises acting on the same, while in a condition having a large surface relative to its mass, with a substantially neutral aqueous solution of hydrogen peroxide until the viscosity characteristics of the nitrocellulose are reduced.

Signed at Rochester, New York, this 11th day of June 1925.

SAMUEL E. SHEPPARD.  
LEON W. EBERLIN.

20

25